

Oct. 14, 1952

R. J. MOORE ET AL

2,614,077

GREASE COMPOSITION

Filed Dec. 27, 1949

FIG. I  
EFFECT OF ADDITIVE CONCENTRATION  
ON ROLL STABILITY OF LITHIUM STEARATE  
GREASE



Inventors:  
Robert J. Moore  
Walfred Saarni  
By James Jodanovic  
their Attorney

## UNITED STATES PATENT OFFICE

2,614,077

## GREASE COMPOSITION

Robert J. Moore, Oakland, and Walfrid Saarni, Berkeley, Calif., assignors to Shell Development Company, San Francisco, Calif., a corporation of Delaware

Application December 27, 1949, Serial No. 135,124

9 Claims. (Cl. 252—33.6)

1

This invention is concerned with the preparation of greases having improved mechanical stability. More particularly, it is directed to grease compositions containing particular classes of agents imparting mechanical stability to greases. In the prior art, numerous lubricating grease compositions have been proposed having various characteristics such as high temperature consistency, resistance to syneresis, resistance to oxidation, water-resistant properties, and the like. As a general rule, such compositions have been prepared by incorporating in a suitable lubricating oil metallic soaps of fatty oils or fatty acids which have the property of thickening the lubricating oil to a grease-like consistency. In many applications of lubricating compositions, the conditions of use are such that liquid compositions are unsatisfactory because they run out of bearings or other parts to be lubricated or they are washed away readily or otherwise rendered ineffective. One of the important characteristics of greases comprises the ability of the composition to maintain its consistency at high temperatures and over extended periods of use. This property is particularly important in ball bearing greases, for example. The ability of the grease to maintain its original consistency can be tested by well known methods which comprise working the grease under standardized conditions and periodically testing its penetration.

The mechanical stability of various greases has been found to vary widely depending principally upon the predominating soap used for gelling the grease. Lithium stearate greases, for example, have been found to have relatively poor mechanical stability. A substantial improvement may be made by substituting, in whole or in part, the fatty acid soap by a soap of a hydroxy fatty acid such as 12-hydroxystearic acid and corresponding acids derived from natural sources such as from hydrogenated castor oil. Where even higher resistance to the adverse influence of the continuous working or elevated temperature is desired, even the soaps of the hydroxy fatty acids of the character described above have been found to be inadequate.

It is an object of the present invention to provide greases having improved mechanical stability. It is another object of the present invention to provide greases having improved mechanical stability at elevated temperatures. It

2

is a further object of the present invention to provide greases having reduced soap content for a given degree of penetration.

Now, in accordance with the present invention, it has been found that greases comprising an oil and 4-25% by weight of two types of soap components, the two soaps being present within a critically defined range of ratios, have outstanding structural stability. The major soap 5 is a lithium soap of an aliphatic monocarboxylic acid having 10 to 24 carbon atoms and bearing no polar groups other than the carboxyl group. The minor soap is that of a monocarboxylic acid having 3 to 18 carbon atoms and bearing a hydrogen bonding substituent less than 9 carbon atoms removed from the carboxyl group. In order to attain the outstanding structural stability with which this invention is concerned, the normal percentage of the minor soap must 10 be between 4 and 12 mole per cent, and preferably, is between 5 and 10 mole per cent, based on the total soap content of the grease.

The stabilizing additives within the purview of the present invention comprise soaps of alkane monocarboxylic acids, cycloalkane monocarboxylic acids and monocyclic aromatic monocarboxylic acids, each of which contains a hydrogen bonding or co-ordinating substituent less than 9 carbon atoms removed from the carboxyl group. The preferred additives which have been 15 found to be especially useful in the present compositions comprise the soaps of alkane hydroxy monocarboxylic acids, the monocycloalkane hydroxy monocarboxylic acids and monocycloaromatic hydroxy monocarboxylic acids. Still other 20 preferred grease additives comprise soaps of monoketoalkane monocarboxylic acids and monoaminoalkane monocarboxylic acids wherein the keto or amino groups are attached to carbon atoms less than 9 carbon atoms removed from the carboxylic acid group.

While the lithium soaps are preferred in the present compositions, other alkali metals such as sodium and potassium may be employed. The class of compounds having outstanding effectiveness in this respect comprises the lithium soaps of monohydroxy alkane monocarboxylic acids having from 3 to 18 carbon atoms wherein the hydroxyl group is in the beta, gamma or delta positions with respect to the carboxyl group, such as hydroxy propionic acids, hydroxy butyric

acids, hydroxy valeric acids, hydroxy caproic acids, hydroxy enanthic acids, hydroxy caprylic acids, hydroxy lauric acids, hydroxy myristic acids, hydroxy palmitic acids, hydroxy stearic acids, and hydroxy arachidic acids, as well as their homologues and analogues. The corresponding mercapto acids wherein the hydroxy group is replaced by a mercapto group function in a similarly effective manner in the present compositions.

Another effective group of stabilizing agents comprises the monoaminoalkane monocarboxylic acid soaps and especially the lithium soaps of acids such as 3-aminopropionic acid, 3-amino-hexanoic acid, 3-aminopentanoic acid, 4-amino-hexanoic acid, 5-aminodecanoic acid, as well as their analogues and homologues. It is preferred that aminoalkane acids having from 3 to 18 carbon atoms be employed and substantially unbranched acids are preferred.

Metal soaps of monoketalkane monocarboxylic acids having from 3 to 18 carbon atoms may be used in the subject greases. These may be lithium, sodium, calcium, aluminum or potassium soaps of acids such as pyruvic acid, propionyl carboxylic acid, acetoacetic acid, levulinic acid and acetobutyric acid. The corresponding thio acids wherein the oxygen atom of the keto group is replaced by a sulfur atom similarly function as stabilizers in the present greases.

A particular type of desirable stabilizer comprises a soap of hydroxy naphthenic acids such as those derived from petroleum sources. It will be appreciated that a mixture of this type is more clearly defined by a source than by its exact structure. However, the hydroxy naphthenic acids which are found to be effective in the present compositions are understood to be predominantly hydroxy alkylated cyclopentanoic acids, a large proportion of which comprises hydroxy derivatives of (3-ethyl-4-methyl-1-cyclopentyl) acetic, butyric and valeric acids. Of course, the pure, clearly defined individual members of this class may be employed if desired. However, mixtures of hydroxy naphthenic acids derived from petroleum oils, when saponified with an alkali metal, function as satisfactory stabilizing agents in these compositions.

The soaps of the aromatic acids which function as mechanical stabilizing agents in the present compositions comprise especially those of monocyclic aromatic monocarboxylic acids bearing a hydrogen bonding or co-ordinating substituent such as a nitro, amino, mercapto, hydroxy, keto, sulfo or thiol group attached to the aromatic ring or to a short side chain thereon. Typical suitable soaps of this description include the sodium, potassium, aluminum, calcium or lithium soaps of ortho-, meta-, or para-nitrobenzoic acid; ortho-, meta-, or para-aminobenzoic acid; ortho-, meta-, or para-thiolbenzoic acid; ortho-, meta-, or para-hydroxybenzoic acid; mandelic acid, tropic acid, benzoyl formic acid and benzoyl acetic acid.

The soaps which function as outstanding stabilizers in the present compositions include those such as described above, especially those of the substituted alkane acids having substantially no branching in the hydrocarbon portion of the molecule as well as the cycloalkane or aromatic acids bearing a minimum of branched chain substituents. The examples appearing hereinafter indicate that the position of the hydrogen bonding or co-ordinating substituent with respect to the carboxyl group is immaterial as long as it is

dependent from a carbon atom less than 9 carbon atoms removed from the carboxyl group. If a greater space exists between the two functional groups, the enhanced mechanical stability of the grease correspondingly suffers.

The class of gelling agents in the greases under consideration comprises the lithium soaps of aliphatic monocarboxylic acids having from 10 to 24 carbon atoms said acids containing no polar substituents other than the carboxyl group. These include especially the mixtures of fatty acids derived from natural fatty oils such as vegetable oils, animal oils, and fish oils. Hydrogenated vegetable oil acids have been found to be especially useful. Other suitable acids include oleic acid, stearic acid, linoleic and linolenic acids, as well as the acids derived from beef fat, tallow and the like.

The lubricant comprising the base of the grease will, in most cases, be a mineral lubricating oil. However, natural oils such as vegetable oils or animal oils may be employed as well as synthetic lubricants such as polymerized olefins, polyalkylene oxides such as polypropylene oxide, polymerized sulfides such as polypropylene sulfide, polymerized glycols such as polypropylene glycol, esters of dicarboxylic acids such as bis-(2-ethylhexyl) sebacate and phosphates such as tributyl phosphate or tricresyl phosphate. In cases where high temperature use is contemplated, fluoro compounds and the hydrocarbyl silicones may be used in whole or in part.

The respective quantities of each of the principal ingredients may be varied within flexible limits except for the required range of ratio of the stabilizing soaps to the principal gelling soaps. While the addition of the stabilizing soaps such as those of 4-hydroxyvaleric acid to soaps such as lithium stearate causes a certain amount of increased mechanical stability, it has been discovered that only within strictly limited ratios an unexpected and surprisingly great increase in mechanical stability is attained. To illustrate this, reference is made to the figure of the drawing accompanying this specification. The figure proves that a critical relationship exists when the stabilizing additives are present in ordinary fatty acid soap greases such as lithium stearate grease. The mole percentage of the additive soap should be between 6 and 12 mole per cent of the total soap content.

The total soap content of the greases may be from about 4 to 25% by weight of the total grease, preferably the soap content is between 7 and 20% by weight of the grease. It will be understood that mixtures may be employed in the case of each of the three principal components. For example, when a low temperature grease is required, up to about 20% by weight of the oil base component is desirably an ester of a dicarboxylic acid such as bis-(2-ethylhexyl) sebacate in admixture with mineral oil. Mixtures of either pure or natural soaps for both the principal gelling agent and for the stabilizer may be used. Other ingredients which may be present in the compositions comprise glycols such as glycerine, for the prevention of bleeding and the like, and anti-oxidants such as para-phenylene diamine. In many instances, additives of this type are found to be unnecessary since the described classes of stabilizing soaps have been found to improve not only the mechanical stability of the grease compositions but also its resistance to bleeding and oxidation.

The preparation of the subject greases prefer-

ably follows the processes described in prior art literature with certain precautions taken to avoid dehydration of the hydroxy stabilizing agents or loss of the other types of hydrogen bonding substituents detailed above. A typical preparation of lithium greases comprises saponification of the two classes of carboxylic acids, namely, the major grease forming fatty acid and the stabilizing acid, dehydration of the soap in the presence of a portion of the oil, solution of the soap in oil by heating, and co-precipitation of the two soaps in the desired fiber form by lowering the temperature, preferably together with stirring and working.

More particularly, it has been found that greases having optimum consistency are prepared by mixing the two types of acids with about one-third of the oil, adding lithium hydrate at about 100° C., then raising the temperature to about 200° C. in order to dehydrate the concentrated soap mixture and to dissolve the soap in the oil. The concentrate is then quenched by the incorporation of the remaining portion of cold oil. The mixture is reheated to about 190° C. and finally cooled to room temperature with working.

The step of dehydration is carried out under conditions which will remove water which has been introduced together with the lithium hydroxide, but heating is controlled, as already indicated, at a temperature lower than the dehydrating temperature of the hydroxy fatty acid or corresponding decomposition temperature of the other stabilizing additives. If the dehydrating temperature is raised above about 230° C., most of the stabilizing additives will gradually lose their hydrogen bonding substituents and form decomposition products principally comprising unsaturated acids or their soaps such as the soaps of acrylic acids or methacrylic acids or their higher homologues. These unsaturated decomposition products, while having certain beneficial effects when present in large amounts, do not have a beneficial effect upon the mechanical stability of greases as described herein when present within the critically defined ratio based on the total soap content. Hence, one feature of the present invention comprises a process of forming the greases of the components discussed above including the step of removing water from the grease at a temperature below the decomposition temperature of the stabilizing additives defined in the foregoing disclosure.

While the mixture of soaps may be preformed and subsequently added to the oil in order to form a grease, it has been found that the quench system provides a grease having far better mechanical stability and, hence, the foregoing described type of formation should be used whenever possible.

While various types of mineral oil may be used in the preparation of the greases of the present invention, it has been found that the more highly refined oils, preferably highly paraffinic and/or naphthenic oils, result in greases having improved mechanical stability when the subject additives are present. Furthermore, the nitrogen content of the refined oil should be as low as possible. Lubricating oils having from 0 to 25% aromatics are especially satisfactory for the present compositions, although the preferred range of aromatic content is that stated hereinbefore.

The mechanical stability of the greases produced in accordance with the present invention may be tested with the Shell Roll Tester cur-

rently used extensively in the grease industry. The apparatus in which the test is made is a simulated roller bearing and consists of a horizontal 3½ inch hollow cylinder, 7 inches long, into which there is placed a solid steel cylinder 2½ inches in diameter and about 7 inches long, weighing approximately 11 pounds. The larger cylinder, initially closed at one end, has a cap placed over the open end after the grease has been introduced. Enough clearance is permitted for the solid steel cylinder to roll freely inside the larger cylinder which is rotated at 160 R. P. M., and the solid cylinder rotates therein by means of contact with the inside of the larger hollow cylinder. In an apparatus of this character, a given amount of grease may be rolled for a period of time and tested for consistency to obtain the degree of mechanical stability of the grease. The smaller cylinder rolls, works and masticates the grease thoroughly during the test. At given time intervals, the grease is removed, tested for consistency and then replaced in the apparatus for further working.

The consistency of the grease is determined by means of a special small cone attached to the regular ASTM penetrometer. A small cup is used in conjunction with the test. The worked penetration obtained by this apparatus is referred to herein as "micro" penetration which may be correlated, if desired, with the regular ASTM penetration by means of a previously determined curve. The roll stability of a grease comprises the time required for rolling in the above apparatus for the grease to reach a maximum micro penetration of 230 dmm.

While the mechanical stability of greases at room temperature is important, it is also imperative that greases have sufficient stability at elevated temperatures if they are to be useful in apparatus running at about 100° C. or even higher. Lithium soap greases are notorious for their poor stability at elevated temperatures. It has been found that the present additives, if they occur in the greases within the critical concentration range discussed above, stabilize the greases sufficiently to permit their use for as much as thirteen times as long a service period as when the unstabilized grease is utilized.

#### EXAMPLE I

In the following tests hydrogenated fish oil acids were employed. These are essentially mixtures of fatty acids with a predominating proportion of stearic acid, and appreciable proportions of other fatty acids having from 14 to 22 carbon atoms. The base oil was a turbine oil of low aromatic content and had a viscosity of 100 centistokes at 100° F., with a viscosity index of 55. One-third of the oil was mixed with the fish oil acids or with fish oil acids and stabilizing acids in proportions to yield a final grease having a total of 8% by weight total soap containing 0.3 weight per cent (8.6 mole per cent) of the stabilizing agent, based on the total composition. Lithium hydrate was added to the mixture at 100° C. in stoichiometric amount to neutralize the acids, after which the soap-oil concentrate was dehydrated at 200° C. The remaining oil was then added and the mass heated to 205-210° C. to dissolve the soaps. The mixture was allowed to cool statically to 120° C., held at this temperature for two hours and then allowed to cool to room temperature. The cooled gel was then worked with an ASTM grease worker to obtain a grease suitable for testing.

The greases prepared by the above process were tested for mechanical stability in the Shell Roll Tester as described hereinbefore. The data in the table show the effect of various additives.

Table

## EFFECT OF ADDITIVES ON MECHANICAL STABILITY OF LITHIUM STEARATE GREASE

| Additive                    | Roll Stability, Hours |
|-----------------------------|-----------------------|
| None                        | Less than 1           |
| Lithium 4-hydroxyvalerate   | 250                   |
| Lithium 4-ketovalerate      | 210                   |
| Lithium 3-hydroxypropionate | 270                   |

An additional feature of the compositions of the present invention comprises the advantage gained with respect to aeration during milling. Under the ordinary conditions of grease milling large amounts of air are incorporated in the grease which must be subsequently removed under vacuum or by some other suitable means. The unmodified grease described above gained 40% in volume during the milling operation. In contrast to this, when any of the other samples containing the stabilizing additives described were milled, the gain in volume due to aeration amounted to about only 4% to 6%. The reason for this improvement in operating characteristics is not obvious at the present time, but the amount of aeration may reflect the formation of extremely fine soap particles by attrition which then function to form an air-oil emulsion.

## EXAMPLE II

Hydrogenated fish oil acids are mixed with 6 mole per cent of alpha-amino-isocaproic acid and mineral lubricating oil. A mixture of soaps is obtained by neutralization of the components with potassium hydroxide. Neutralization is effected by heating a mixture of oil, hydroxide and acids. The composition may be dehydrated at a temperature of about 100-200° C. Sufficient additional oil is added and the mixture is milled to give a grease having a total soap content of about 10%. Greases prepared in accordance with this procedure have excellent mechanical stability.

We claim as our invention:

1. A lubricating grease having approximately the following composition:

|                                              | Approximate weight per cent |
|----------------------------------------------|-----------------------------|
| Mineral lubricating oil                      | 92.0                        |
| Lithium soaps of hydrogenated fish oil acids | 7.7                         |
| Lithium soap of 4-hydroxyvaleric acid        | 0.3                         |

2. A lubricating grease having approximately the following composition:

|                                              | Approximate weight per cent |
|----------------------------------------------|-----------------------------|
| Mineral lubricating oil                      | 92.0                        |
| Lithium soaps of hydrogenated fish oil acids | 7.7                         |
| Lithium soap of 4-ketovaleric acid           | 0.3                         |

3. A lubricating grease composition containing only carboxylic acid soaps as gelling agents comprising a major amount of a mineral lubricating oil having an aromatic hydrocarbon content between 0 and 25% by weight and between 4 and 25% by weight of a mixture of alkali metal soaps of aliphatic monocarboxylic acids, at least one of said soaps being a lithium soap of an acid having from 12 to 24 carbon atoms and bearing

no polar substituents other than the carboxyl group and at least another one of said soaps being an alkali metal soap of an acid being a hydroxy fatty acid having from 3 to 18 carbon atoms, wherein the hydroxy substituent is less than 9 carbon atoms removed from the carboxyl group, said hydroxy fatty acid soap constituting from 4 to 12 mole per cent of the total soap content.

5 10 4. A lubricating grease composition containing only carboxylic acid soaps as gelling agents comprising a major amount of a mineral lubricating oil, 4 to 25% by weight of the grease of a mixture of lithium soaps of fatty acids, at least one

15 15 of said acids having from 12 to 24 carbon atoms, and at least another one of said acids being a hydroxy fatty acid having from 3 to 18 carbon atoms, the hydroxy substituent being less than 9 carbon atoms removed from the carboxyl group, said soaps of the hydroxy fatty acid constituting between 5 and 10 mole per cent of the total soap content.

20 20 5. A grease composition containing only carboxylic acid soaps as gelling agents comprising a lubricating oil, 4 to 25% by weight of a mixture of lithium soap of an aliphatic monocarboxylic acid having 10 to 24 carbon atoms bearing no polar groups other than the carboxyl group, and an alkali metal soap of an aliphatic

30 30 monocarboxylic acid having 3 to 18 carbon atoms bearing a hydrogen bonding substituent less than 9 carbon atoms removed from the carboxyl group, the second soap being present in an amount between 4 and 12 mole per cent of the total soap content.

35 35 6. A grease composition containing only carboxylic acid soaps as gelling agents comprising a lubricating oil, 4 to 25% by weight of a mixture of lithium soap of an aliphatic monocarboxylic acid having 10 to 24 carbon atoms bearing no polar groups other than the carboxyl group, and an alkali metal soap of a monocarboxylic acid having 3 to 18 carbon atoms bearing a hydrogen bonding substituent less than 9 carbon atoms removed from the carboxyl group,

40 40 the second soap being present in an amount between 4 and 12 mole per cent of the total soap content, said hydrogen bonding substituent being one selected from the group consisting of hydroxy, keto, amino, nitro, mercapto, thiol and sulfo groups.

45 45 6. A grease composition containing only carboxylic acid soaps as gelling agents comprising a lubricating oil, 4 to 25% by weight of a mixture of lithium soap of an aliphatic monocarboxylic acid having 10 to 24 carbon atoms bearing no polar groups other than the carboxyl group, and an alkali metal soap of a monocarboxylic acid having 3 to 18 carbon atoms bearing a hydrogen bonding substituent less than 9 carbon atoms removed from the carboxyl group,

50 50 the second soap being present in an amount between 4 and 12 mole per cent of the total soap content, said hydrogen bonding substituent being one selected from the group consisting of hydroxy, keto, amino, nitro, mercapto, thiol and sulfo groups.

55 55 7. A grease composition, containing only carboxylic acid soaps as gelling agents, comprising a lubricating oil and from 4 to 25% by weight of a mixture of a lithium soap of a fatty acid having from 10 to 24 carbon atoms per molecule and a

60 60 lithium hydroxy propionate, the latter being present in an amount between 4 and 12 mole per cent of the total soap and salt content.

65 65 8. A grease composition, containing only carboxylic acid soaps as gelling agents, comprising a lubricating oil and from 4 to 25% by weight of a mixture of a lithium soap of a fatty acid having from 10 to 24 carbon atoms per molecule and a lithium soap of a keto fatty acid having from 3 to 18 carbon atoms per molecule, the keto group being less than 9 carbon atoms removed from the carboxyl group, the latter soap being present in an amount between 4 and 12 mole per cent of the total soap content.

70 70 9. A grease composition, containing only carboxylic acid soaps as gelling agents, comprising

a lubricating oil and from 4 to 25% by weight of a mixture of a potassium soap of a fatty acid having from 10 to 24 carbon atoms per molecule and a potassium soap of an amino fatty acid having from 3 to 18 carbon atoms per molecule, the amino group being less than 9 carbon atoms removed from the carboxyl group, the latter soap being present in an amount between 4 and 12 mole per cent of the total soap content.

ROBERT J. MOORE. 10  
WALFRID SAARNI.

## REFERENCES CITED

The following references are of record in the file of this patent:

## UNITED STATES PATENTS

| Number    | Name           | Date           |
|-----------|----------------|----------------|
| 2,450,254 | Puryear et al. | Sept. 28, 1948 |
| 2,455,892 | Fraser         | Dec. 7, 1948   |
| 2,468,098 | Morway et al.  | Apr. 26, 1949  |
| 2,487,080 | Swenson        | Nov. 8, 1949   |